

Oct. 26, 1954

J. B. BRENNAN

**2,692,411**

## METHOD OF CONTINUOUS CASTING

Filed March 12, 1951

Fig. 1



Fig. 3



Fig. 4



Fig. 5



Fig. 2



INVENTOR.  
Joseph B. Remsen

## UNITED STATES PATENT OFFICE

2,692,411

## METHOD OF CONTINUOUS CASTING

Joseph B. Brennan, Cleveland, Ohio

Application March 12, 1951, Serial No. 215,096

2 Claims. (Cl. 22—200.1)

1

This invention relates to continuous casting whereby a lamination of two or more metal strips or shapes is produced by passing a carrier mold and one or more metal objects or strips to be laminated through a body of molten metal and a heating zone and subsequently through a forming and solidification die.

According to my invention, a lamination of metal may be applied continuously to another metallic article, the article on which the lamination is applied being in tubular, strip or other form.

It is also to be understood that the principles of the invention may be applied and the objects thereof may be achieved in the casting of ceramic material, quartz, mica, germanium, silicon, glass, and other fusible materials, as well as in the casting of metals. For example, a lamination of ceramic material may be applied to a metallic base material, or a metallic material may be applied to a ceramic base material, it being possible according to my invention to laminate any base material having a melting point higher than the melting point of the material from which the lamination applied thereto is cast, the cast material, in the case of a metal cast around a ceramic core, adhering around said core by shrinkage and to some extent by flow of the metal into any surface irregularities and pores of said core. Of course where a chemical bond is desired, well known bonding agents may be employed between the metal and ceramic.

Insofar as common subject matter is concerned, this application constitutes a continuation in part of my pending applications Serial No. 147,466, filed February 18, 1950; Serial No. 201,171, filed December 16, 1950; and Serial No. 202,707, filed December 26, 1950, and Ser. No. 25,756, filed May 7, 1948, now Patent No. 2,569,150 granted September 25, 1951.

In my prior patent applications aforesaid, I described in detail a method of casting whereby a carrier core or mold is passed through a pool of molten material and through an adjacent cooling die; and, in these applications, I described the various means and modifications whereby various shaped objects could be cast. In this, my present invention, I propose a method of casting whereby a laminated product may be obtained in a simple and efficient manner using similar principles.

A feature of this invention is the continuity which may be obtained by my laminated casting method.

A further feature of my invention is the passage of the carrier mold and the article to which

2

the lamination is to be applied through the body of molten material and an adjoining forming and solidification die after having the lamination cast thereon.

Another object of my invention is to cast a laminated object in accurately controlled dimensional sizes.

A further advantage of my invention is the saving in cost which I effect by the practice of the invention and the ease by which I obtain laminated casting highly desirable for use in the metal art field, such as, for example, in bearing manufacture.

Further objects and advantages of my invention will become more apparent as a description of the drawings proceed.

To the accomplishment of the foregoing and related ends, said invention, then, comprises the features hereinafter fully described and particularly pointed out in the claims, the following description and the annexed drawings setting forth in detail certain illustrative embodiments of the invention, these being indicative, however, of but a few of the various ways in which the principal of the invention may be employed.

Referring now to the drawings annexed hereto.

Figure 1 is a sectional and elevational view of apparatus whereby the method of my invention may be practiced;

Figure 2 is a cross sectional view of a tubing or bushing which may be obtained by the practice of the method illustrated in Figure 1.

Figure 3 is a cross sectional view of another type of mold and the article thereby secured according to my invention; Figure 4 is a variation of Figure 3.

Figure 5 illustrates a laminated strip obtainable by the practice of my invention.

Further referring to Figure 1, the mandrel or carrier mold 2 is passed through the bearing sleeve 3 located upon the extending arm 1 which is attached, for example, to the crucible 5 at the point 4. As the mandrel or carrier mold 2 is passed downward through the bearing sleeve 3, the metallic sheet 6 is unwound from the drum 7 rotating upon the axle 8 and is moved downward over the guide wheels 9 which direct the metallic sheet 6 toward and around the mandrel or carrier mold 2. The rollers 10 complete the tubular forming process of the metallic sheet 6 around the mandrel or carrier mold 2.

If preferred, the tubular form 6 may be made and fed down without the core 2 moving and the core 2 may be of metal or ceramic material.

The carrier mold or core 2, instead of being

in the form of a cylindrical mandrel, may be square, rectangular, triangular, or it may be of other flat or curved or angular sided shape. This will permit the utilization, for example, of an entire width of steel; also, if desired, it will facilitate slitting of the laminated article into flat strips. In preference to the steel drum 1 and the rollers 9 and 10, it is possible in the practice of the method herein disclosed to form the metal 6 around the carrier mold 2 in the manner heretofore described in my prior applications. In such instance, the sheet 6 would be cast around the carrier mold 2 by passage of the mold 2 through a body of molten metal and subsequently through a forming and solidification die and after the sheet 6 has been cast about the mold or core 2, the mold 2 with the sheet 6 cast therearound is then passed through the second molten metal pool 11 in the crucible 5 in the manner herein-after more fully described.

The mandrel or carrier mold 2 may be made of an investment such as, for example, zirconium oxide, graphite, or molding plaster or a heat resisting metal. Among other well known materials, core sand, molding sand binders and carbon also may be used to make the molds. The mold may consist of an annular ring such as illustrated in my applications Serial Nos. 147,466 and 202,171; or it may consist of a straight piece such as is shown in my application Serial No. 202,707. Or the mold may consist of a series of divisible molds stacked in aligned relationship in a manner such as is shown in my application Serial No. 202,707 aforesaid.

Further the mandrel, or core form 2 which is fed through the pool of molten metal may be destructible or it may be of a permanent core or mold nature. After the sheet 6 has been formed around the moving carrier core 2 by the rolls 10, the carrier core 2 and encompassing sheet 6, for example, are further moved downward into the body or pool of molten metal 11. The temperature of the molten metal 11 and the sheet 6 is maintained by the electro-conductive coils 12. As the carrier mold or mandrel 2 and the sleeve form 6 pass through the molten metal 11 the molten metal fills in around and passes into the forming and solidification die 14. The sheet 6 and the sleeve 6 become heated to the temperature of the molten metal 11. The outside of formed metal base 6 is spaced a distance which corresponds to the thickness of the desired laminated layer 13 provided between the outer surface of the sheet 6 and the inner surface of the forming and solidification die 14 and is guided centrally therein. As the heated formed metallic sheet 6 and the molten metal 11 therearound further proceed downward into and through the forming and solidification die 14, the molten metal 11 is solidified and thermally bonded to the steel, and the laminated layer 13 is bonded over and around the sheet 6. The solidification portion 14b of the die 14 is controlled, for example, in temperature by the exterior cooling coils 15a located in the cooling die 15. Alternatively, other cooling means may be employed for purposes of this invention. As the mold 2, the metal layer 6, and the laminated layer 13 complete their passage through the forming and solidification die 14, inside the cooling die 15, the desired lengths may be cut off by means of the cut off tool 16. In any event the laminated layer is pre-formed in a molten condition around the metal to be laminated and solidified thereon. Cooling means may also be incorporated inside mandrel 2,

In the particular example of the invention which I have described in Figure 1, it should be understood that a guide tube or unit molds (not shown) such as I have disclosed in my application Serial No. 202,707, filed December 26, 1950, also may be adapted to the process of this invention. The splines to which I have made reference therein may also be used herein for purposes of guiding the carrier mold or core 2 through the body of molten metal and aligning the carrier mold or core 2 with the metallic sheet form 6 thereon with reference to the forming and solidification die. Here again, if it is desired to produce laminated strip material where a central mold is employed, the splines may extend into the zone of solidification, the splines here also being spaced apart a distance corresponding the desired width of the laminated cast strip. The splines may be employed with or without a clearance allowance for fins between the strips. Where no allowance is made for these fins, a tension means is desirable in order to aid the withdrawal of the strips from the solidification die.

The cast metal lamination may be applied to the inside or outside, or only partially to a surface, or it may be applied to both surfaces of a tubular, flat, or rod, or other shape material. Where a tube is cast, the resultant tube may be opened and flattened or otherwise re-shaped, such as by reforming it to enclose the externally deposited and bonded metal on the inside.

Also when a lamination is cast externally over or on a piece of steel, as is shown in Figure 1, the laminated product may be divided into one or more strips prior to lamination, or it may be split open on the seam and flattened out after lamination.

The distance of heat application above the cooling zone may be regulated to the rate of cooling. Lengthwise chilling may be effected by endwise cooling. Also, the distance of travel while enclosed in the solidification zone may be regulated.

As has been previously explained, the tube 6 may be cast in a preceding crucible casting setup. This arrangement is particularly desirable where a laminated seamless tubing is wanted.

It is also to be understood that laminated bushings may be manufactured according to the method described herein, in a manner similar to that described in my application Serial No. 202,707, filed December 26, 1950.

It must be understood that it is possible to make continuous laminated tubing according to this invention and that it is possible to produce bushings or other metallic objects. The length of the finished laminated product can be controlled by means of the cut off tool 16.

A particular example of my invention resides in the fact that there is a forming section for the cast fluid metal. This forming section lies above the solidification zone and beneath the molten metal pool, and is indicated at 14a in Figure 1, the formed lamination prior to solidification being indicated at 13a. However, where a guide tube is employed, this forming section may extend up into the molten metal pool itself.

It is also possible to produce laminated tubing according to my invention by having the core mandrel 2, Figure 1, stationary and ending at the point shown by the diametric dotted line below the cooling die 14, Figure 1, in which modification the produced lamination will be withdrawn by tension rolls or other means not shown below the solidification zone 15 and outside thereof.

It is also possible according to my invention to have mandrel 2, Figure 1, rectangular or square or other shape and to draw strips thereover through the pool of molten metal and thereby cast and bond a lamina of molten metal on each strip.

It is also possible to modify the forms shown in Figure 3 and Figure 4 so as to enclose the core 2 of Figure 1 having cast or applied metal over core 2 and to use the half molds of Figure 3 and Figure 4 as enclosures for a single or double layer of metal cast about core 2. In this variation the forms 20 and 21 of Figure 3 and Figure 4 would be hollow half cylindrical shells and pass through the molten pool 11, Figure 1, guided and spaced around core 2 and thereafter in exterior contacting relationship with the cooling die 14 and have the cast tubular metal therein in single or double layer as desired. This arrangement could be used with core 2 moving or stationary and ending just below cooling zone 15, Figure 1. In this way it is possible to cast tubing continuously of single or double thickness. It is necessary to have 2 pools of molten metal and the solidification zones associated therewith one over the other to cast a double layer of metal tubing. In this case the core 2, Figure 1, may be stationary or moving as explained above.

In the practice of my invention wherein a metal lamination is applied to a metallic material, the base metal to which the lamination is applied has a melting point higher than that of the metal employed for the lamination casting.

Referring to Figure 2, the finished product produced by the method and apparatus of Figure 1 is shown in cross section. The metallic sheet 6 has the laminated layer 13 thereover. The slit 17 in the metallic sheet 6 can be eliminated, where desired, by a prior passage of the formed sheet 6 through a welder to weld the edges of the seam and thereafter casting the strip 6 therearound.

In Figure 3, I have illustrated a further adaptation of my invention. In this instance the metallic strips 18 and 19, as of steel, for example, are located within and edge gripped if desired by the opposed aligned sectionalized carrier mold parts 20 and 21. This type of mold is similar to that described in my application Serial No. 201,171, filed December 16, 1950, and may consist of two annular rings or two straight pieces; the practice of the method with this type of mold is similar to that previously described in my application Serial No. 202,707, filed December 26, 1950. The strips 18 and 19 are located within the opposed aligned molds 20 and 21 and are passed through guides and beneath the surface of the molten metal 11 in the crucible 5. Passageways 27 and 28 are shown which extend from the exterior of the carrier molds 20 and 21 to the cavities defined by the complementary portions of the molds 20 and 21 and the metallic strips 18 and 19. These passageways may be constructed in any conventional manner, and as heretofore have been described in my aforesaid applications. The molten metal then flows into the cavities located between the strips 18 and 19 and the interior of the molds 20 and 21. Thereafter, the strips 18 and 19 and the molds 20 and 21 are passed through the die 14 with its exterior cooling section 15 whereupon the cast facings or laminations 22 and 23 is solidified. Upon solidification there are formed the laminated layers 22 and 23, for example, of bronze. When

5  
the mold sections 20 and 21, securely holding the steel strips 18 and 19 therebetween, are passed through the pool of molten metal 11 and the high frequency field created by the coil 12, the steel strips become heated to a bonding temperature so that when the metal laminations 22 and 23 are cast thereagainst, a good bond is obtained. A temperature from 2100° F. to 2300° F. is generally suitable when applying bronze to steel. In effect according to the apparatus shown in Figure 3, it is possible to pass two straight carrier bars or molds 20 and 21 which correspond to the carrier mold or mandrel 2 in Figure 1 through the molten metal pool 11 and then through the so forming and solidification die 14.

Figure 4 illustrates a method similar to that described in reference to Figure 3. In this instance a single metallic strip 24, as of steel, is located between and held by the complementary portions of the opposed aligned molds 20 and 21. The molten metal here flows into the molds 20 and 21 through openings 27 and 28 and the laminated facings 22 and 23 are cast and formed on the opposed surfaces of the strip 24 in a single operation.

20  
25  
30  
35  
40  
45  
50  
55  
60  
65  
70  
75  
The mold halves 20 and 21 in Figures 3 and 4 and the core 2, Figure 1, may be carried by chains or hydraulic pushers through the molten metal pool 11 and the forming zone 14a and through the solidification zone 14, Figure 1, for the purposes of this invention.

Figure 5 illustrates a laminated cross-sectional strip which may be produced according to this invention and consists of a single metallic strip 25, as, for example, steel with the cast lamination 26 of, for example, bronze bonded thereto. The article of Figure 5 may be produced according to the method described in reference to Figures 3 and 4 and 1. The strip 25 in this instance extends a distance equivalent to the diameter of the molds 20 and 21. The laminated layer 26 cast thereon corresponds in width to the width of the strip 25. In this case, the lamination is applied to only one face of the base steel strip. Spline and center spacing guides may be used in the molten metal pool and above it to align the steel strip and the mold sections.

In some cases it may be desirable to pass solid cast tubing or welded tubing through the pool of molten metal for lamination. In some cases it may be desirable to coat between the inside and the exterior surface of steel tubing for example with laminated metal. This can be done by extending the depth of the metal 11, Figure 1, and the crucible 5, Figure 1, and the high frequency coil 12, Figure 1, upward to encompass and enclose rolls 10, Figure 1, and by reducing the diameter of the mold from 2 and holding it in interspaced relationship from the steel 6 to permit the molten metal to flow inside the steel strip 6 as it is formed about the mold 2.

In case the molten metal is cast inside the steel strip 6 as it is being formed about the mold 2, this zone preferably must be kept above the melting point of the metal being cast. The mold 2 in this case should terminate in the cooling zone in case it is stationary, to reduce the friction due to shrinkage of the cast metal about the mold 2. The mold 2 may also in this instance be reduced in diameter by tapering progressively as it extends down through the cooling zone to eliminate adherence of the cast metal thereto.

Other means of introducing the metal to the interior as well as to apply it to the exterior and to bond the metal thereto will be apparent to

those skilled in the art because of the principles which I have taught herein, the above examples being illustrative only of some methods of accomplishing the result of my invention.

It is also to be understood that the apparatus of this invention may be enclosed in variable pressure apparatus (not shown) such as is disclosed and described in my pending application Serial No. 202,707, filed December 26, 1950, and my prior Patent No. 2,371,604, issued March 20, 1945. Such variable pressure apparatus very readily may be employed in conjunction, for example, with the apparatus of Figure 1. Where such variable pressure apparatus is used to practice the art of my invention, the lamination casting disclosed herein then may be carried out under pressure or vacuum or under a controlled atmosphere in much the manner described in my application Serial No. 202,707 aforesaid.

It is possible with the apparatus and by the method of my invention to cast oxygen free metal laminations. The air of the atmosphere or other gaseous impurities may be removed and a vacuum created in the variable pressure apparatus, and where it is desired to, cast under a pressure other than that of a vacuum, an inert gas may be supplied to the variable pressure apparatus. Impurities, such as oxides, can be reduced and converted into pure metal by bubbling a deoxidizing gas, such as carbon monoxide, through the molten metal in the manner described in my Serial No. 202,707 aforesaid. In addition, a vacuum may be used to remove or to aid in the removal of the gaseous impurities from the molten metal or to eliminate the presence of free oxygen in the variable pressure chamber.

It is to be understood that the base or core 2 may be stationary and need not move with the base material 6 to which the lamination is to be applied. In this instance, the stationary core passes through the crucible containing the molten material and only through the forming and solidification die.

It will be understood that the invention is not limited to the specific examples set forth since modification may be resorted to within the scope of the invention.

Having thus described my invention what I claim is:

1. A method of producing laminated material from a strip of material and a pool of molten metal contained in a vessel having an open-ended die below the level of the molten metal in the vessel and a laterally fixed, relatively rigid mandrel projecting into said die in accurately spaced relation thereto, comprising forming a hollow member on said mandrel from strip material, which forms one lamination of the finished material, moving the member, guided by said mandrel into and through the pool to heat the member to a bonding temperature and continuing the guided movement of said member into said die, where the second laminating element solidifies on the member.

2. A method of producing laminated material from a strip of material and a pool of molten metal contained in a vessel having an open-ended die below the level of the molten metal in the vessel and a laterally fixed, relatively rigid mandrel projecting into said die in accurately spaced relation thereto and projecting through the vessel, comprising forming a hollow member from strip material, which forms a laminating element of the finished material, moving the member, guided by said mandrel, into and through the pool to heat the member to bonding temperature, continuing the guided movement of said member into said die, where the second laminating element solidifies on the member, and longitudinally splitting and flattening the composite member and solidified laminating element to produce laminated material in strip form.

References Cited in the file of this patent

UNITED STATES PATENTS

| Number    | Name             | Date           |
|-----------|------------------|----------------|
| 124,911   | Newton           | Mar. 26, 1872  |
| 1,995,258 | Stockfleth       | Mar. 19, 1935  |
| 1,999,114 | Sherwood         | Apr. 23, 1935  |
| 2,055,980 | Liebmann         | Sept. 29, 1936 |
| 2,092,284 | McCarroll et al. | Sept. 7, 1937  |
| 2,128,942 | Hudson           | Sept. 6, 1938  |
| 2,338,781 | Porter           | Jan. 11, 1944  |